

# United States Patent Office

2,785,040

Patented Mar. 12, 1957

1

2,785,040

## PROCESS FOR DYEING CELLULOUS MATERIALS WITH METALLIZABLE DIRECT DYESTUFFS AND ANIONS OF A POLYPHOSPHORIC ACID

Jean Gross, Karl Menzi, and Jacques Wegmann, Basel, Switzerland, assignors to Ciba Limited, Basel, Switzerland, a Swiss firm

No Drawing. Application December 12, 1952,  
Serial No. 325,716

Claims priority, application Switzerland  
December 14, 1951

14 Claims. (Cl. 8—42)

This invention is based on the observation that cellulose-containing materials can be dyed in an advantageous manner with metallizable direct dyestuffs, which form sparingly soluble metal complexes, by adding an agent yielding metal to a bath containing a small quantity of non-metallized dyestuff, if there is used as an agent yielding metal an agent yielding nickel or copper and the metallization is carried out in a neutral to alkaline medium in the presence of anions of a polyphosphoric acid.

The dyestuffs used in the present process contain as metallizable groups, for example, ortho-hydroxy-carboxylic acid (salicylic acid), ortho:ortho'-dihydroxy-azo- or ortho - hydroxy - ortho' - carboxy - azo-groupings or 8-hydroxyquinoline radicals. There come into consideration exclusively those direct dyestuffs, that is to say, dyestuffs suitable for dyeing cellulose-containing materials by the usual direct dyeing methods, of which the complex nickel or copper compounds prepared in substance are so sparingly soluble in water themselves and in the form of their alkali salts that they cannot be used for dyeing by the usual methods from an alkaline bath without special assistants. These metallizable dyestuffs are advantageously used in the present process in the form of their alkali salts. In some cases it is desirable to dissolve the dyestuff with the addition of an alkali, for example, an alkali carbonate or alkali hydroxide. A large excess of an alkali hydroxide is, however, preferably avoided as it may have a disadvantageous effect.

As agent yielding metal there come into consideration agents yielding nickel and especially those yielding copper. The agent yielding metal is added to the dyebath after or at the earliest simultaneously with the addition of the compound providing anions of a polyphosphoric acid.

As agents yielding metal there may be used, for example, simple water-soluble salts of nickel or copper, that is to say, those which do not contain the metal in complex union, such as nickel sulfate or copper sulfate. In this form of the process there are advantageously used as compounds providing the anions of a polyphosphoric acid, alkali salts of polyphosphoric acids of the formula



in which  $m$  represents a whole number greater than one. Especially valuable are tetra-alkali pyrophosphates, for example, tetra-sodium pyrophosphate ( $Na_4P_2O_7 \cdot 10H_2O$ ). These alkali pyrophosphates may be added to the dyebath at the outset, if desired, as an alkaline addition for dissolving the dyestuff (see above), or after the material to be dyed has been entered in the dyebath, but at the latest simultaneously with the agent yielding metal.

A procedure that is especially advantageous in many cases is to use as the agent yielding metal an alkali-nickel pyrophosphate or alkali-copper pyrophosphate, for example, sodium-copper pyrophosphate ( $3Na_4P_2O_7 \cdot Cu_2P_2O_7$ ). As these compounds contain, in addition to the metal forming the complex, the residue of pyrophosphoric acid, the

2

further addition of a phosphorus compound of the above kind is unnecessary.

In order to utilize the improvement in tintorial properties brought about by the metallization of the dyestuff and to ensure always producing the same tint with the same dyestuff, there is used at least the theoretical quantity of the agent yielding metal required for complete metallization, and advantageously an amount in excess of this quantity, for example, a total amount of up to twice the theoretical quantity.

The quantity of the polyphosphoric acid ions in the dyebath has a certain influence on the result. In order to avoid the precipitation of insoluble copper compounds, the dyebath should contain at least 2 mols of pyrophosphate ions per gram-atom of copper (which corresponds to the constitution of the sodium-copper pyrophosphate mentioned above). Provided that the excess of the agent yielding copper, calculated on the quantity of dyestuff used, is not inordinately high and amounts, for example, to about 100 percent, it is desirable to make up the dyebath so that it contains at most 8 mols of pyrophosphate ions per gram-atom of copper. A higher content of pyrophosphate ions may lead to incomplete metallization. From this fact, and from the observation that with a large excess of pyrophosphate ions but with the same quantitative ratio of copper to pyrophosphate ions the incomplete metallization occurring under the usual conditions can be considerably improved by a substantial increase in the quantity of the agent yielding copper (and a corresponding increase in the amount of pyrophosphate), calculated on the quantity of dyestuff it can be concluded that a kind of equilibrium reaction is involved.

In dyeing cellulose-containing materials with direct dyestuffs the dyestuff, as is generally known, is not fixed on the goods to the extent of 100 percent, but a certain residue, which in some cases is quite small, always remains unused dissolved in the dyebath, although the dyeing process appears to be practically complete. At this stage of the dyeing process the metallization of the invention can generally be brought about, that is to say, the agent yielding copper may be added. Whether it is possible without disadvantage, or may even be of advantage, to add the agent yielding metal beforehand, depends mainly on the constitution of the dyestuff and in part on the concentration of the bath. With some dyestuffs it is possible to add the agent yielding metal when the dyestuff is only partially fixed on the fiber. In the case of a number of dyestuffs the dyeing may be carried out by adding the agent yielding metal at the outset, for example, it may be added to the dyebath before the material to be dyed is entered.

As has been briefly mentioned above, the dyestuffs are advantageously used in the form of their alkali salts. This applies also to the examples of the process given above, although in the examples the dyestuffs, as is usual, are formulated in the form of the free acids. The dyestuffs can be made up to the desired strength with the usual agents each, for example, as sodium sulfate, sodium carbonate, urea, saccharose or dextrin. If this standardization to a predetermined strength is carried out with a sufficient quantity of an alkali pyrophosphate, no further pyrophosphate need be added for dyeing, and the metallization can be carried out merely by adding at the appropriate moment a simple metal salt such, for example, as copper sulfate, without any other addition.

In other respects the dyeing is carried out by one of the methods known for direct dyeing dyestuffs at a raised temperature, for example, in a boiling bath or near the boiling point, and advantageously with the addition of one of the usual salts, such as sodium sulfate.

In certain cases it may be of advantage to after-treat

dyeings produced by the present process with agents which enhance their properties of wet fastness. In this connection there may be mentioned, for example, treatment with a reaction product of formaldehyde with a compound such as cyanamide, dicyanamide, dicyandiamide or melamine. There may also be mentioned after-treatment agents which are prepared without formaldehyde.

As will be evident from the foregoing description the dyeing and the metallization in the present process take place in the same bath. Among the known methods in which this is possible, only those have been of practical importance hitherto in which metallization is carried out in the presence of an aliphatic hydroxy-carboxylic acid, especially tartaric acid. However, in contradistinction to the present process, it is hardly possible with the known methods to produce useful dyeings when the agent yielding metal is added before the greater part of the dyestuff has been absorbed. The present process possesses quite generally the surprising advantage that aliphatic hydroxy-carboxylic acids are not required, and the much more readily accessible polyphosphates can be used with at least equal success.

The following examples illustrate the invention, the parts and percentages being by weight unless otherwise stated, and the relationship between parts by weight and parts by volume being that of the kilogram to the liter:

*Example 1*

1 part of the dyestuff of the formula



and 0.1 part of sodium hydroxide solution of 30 percent strength are covered with 100 parts of water, and the

4 mixture is raised to the boil. A dyebath is prepared by diluting the resulting stock solution with 2900 parts of water having a temperature of about 60° C.

5 20 parts by volume of an aqueous solution containing in 100 parts by volume 10 parts of sodium-copper pyrophosphate are added to the dyebath. 100 parts of previously wetted cotton are then entered, and the bath 10 temperature is raised to the boil in the course of 1/2 hour. Boiling is carried on for 3/4 hour, during which 15 20 parts of crystalline sodium sulfate are added after 10 minutes and a further 20 parts thereof after 20 minutes. At the end of this period the dyebath is well exhausted. The dyeing is rinsed in the cold, centrifuged and dried. 15 There is obtained a deep blue dyeing of good fastness to light and washing.

A similar result is obtained if the sodium-copper pyrophosphate is added during the exhaustion of the dyebath or only at the end of the exhaustion.

20 By using, instead of the aforesaid sodium-copper pyrophosphate solution, the same quantity of a solution of 4.28 parts of crystalline copper sulfate and 15.4 parts of tetrasodium pyrophosphate ( $Na_4P_2O_7 \cdot 10H_2O$ ) in 90 parts of water, the dyeing process gives a similar result.

25 A similar result is obtained by using, instead of sodium-copper pyrophosphate, sodium-nickel pyrophosphate or an equivalent quantity of a mixture of nickel sulfate and tetrasodium pyrophosphate.

30 Instead of dyeing with the dyestuff of the above formula

cotton may be dyed in the same manner with the following dyestuffs:

|        | Dyestuff of the formula | Tint of dyeing                          |
|--------|-------------------------|-----------------------------------------|
| 1..... |                         | {Cu: Reddish grey.<br>Ni: Reddish grey. |
| 2..... |                         | {Cu: Grey.<br>Ni: Navy blue.            |
| 3..... |                         | {Cu: Reddish grey.<br>Ni: Violet.       |
| 4..... |                         | {Cu: Brown.<br>Ni: Brown.               |

| Dyestuff of the formula |  |  | Tint of dyeing                                               |
|-------------------------|--|--|--------------------------------------------------------------|
| 5.....                  |  |  |                                                              |
| 6.....                  |  |  | {Cu: Blue.<br>{Ni: Reddish blue.<br>{Cu: Blue.<br>{Ni: Blue. |

The sodium-copper pyrophosphate is prepared as follows:

44.6 parts of crystalline sodium pyrophosphate are dissolved in 300 parts of hot water, and the solution is added to a solution of 51 parts of crystalline copper sulfate ( $\text{CuSO}_4 \cdot 5\text{H}_2\text{O}$ ) in 200 parts of water. There is formed immediately a white precipitate of copper pyrophosphate, which is filtered off and washed with water.

The resulting copper pyrophosphate is introduced into a boiling solution of 134 parts of crystalline sodium pyrophosphate in 150 parts of water, and boiling is continued until dissolution is complete. The deep blue, clear solution is evaporated in vacuo, and the easily water-soluble sodium-copper pyrophosphate ( $3\text{Na}_4\text{P}_2\text{O}_7 \cdot \text{Cu}_2\text{P}_2\text{O}_7 \cdot 3\text{H}_2\text{O}$ ) is obtained in the form of a pale powder.

Sodium nickel pyrophosphate is prepared in the same manner with the corresponding equimolecular quantities of nickel sulfate and sodium pyrophosphate.

#### Example 2

1 part of the dyestuff, obtained by reducing the nitro-disazo-dyestuff of the formula



with glucose in sodium hydroxide solution, and 0.1 part of sodium hydroxide solution of 30 percent strength are covered with 100 parts of water, and the mixture is boiled. By diluting the resulting stock solution with 2900 parts of water having a temperature of about 60° C. a dyebath is prepared.

100 parts of previously wetted cotton are entered and the bath temperature is raised in the course of 1/2 hour to 100° C. Boiling is continued for 3/4 hour, during which 20 parts of crystalline sodium sulfate are added after 10 minutes and a further 20 parts thereof after 20 minutes. At the end of this period there are added to the dyebath 20 parts by volume of an aqueous solution containing in 100 parts by volume 10 parts of sodium-copper pyrophosphate, and the treatment is continued for 30 minutes. The dyebath is well exhausted. The dyeing is rinsed in the cold, centrifuged and dried. There is obtained a grey dyeing of good fastness to light and washing.

A similar result is obtained by adding the sodium-copper pyrophosphate to the dyebath at the beginning of the dyeing operation.

By using, instead of the aforesaid solution of sodium-copper pyrophosphate, the same quantity of a solution of 4.28 parts of crystalline copper sulfate and 15.4 parts of crystalline tetrasodium pyrophosphate in 90 parts of water, the dyeing process gives a similar result.

crystalline tetrasodium pyrophosphate in 90 parts of water, the dyeing process gives a similar result.

A similar result is obtained by using, instead of sodium-copper pyrophosphate, sodium nickel pyrophosphate or an equimolecular mixture of nickel sulfate and tetrasodium pyrophosphate.

#### Example 3

1 part of the dyestuff of the formula



and 0.1 part of sodium hydroxide solution of 30 percent strength are covered with 100 parts of water, and the mixture is boiled. A dyebath is prepared by diluting the resulting stock solution with 2900 parts of water having a temperature of about 60° C.

100 parts of previously wetted cotton are entered and the temperature of the bath is raised to 100° C. in the course of 1/2 hour. Boiling is continued for 3/4 hour, during which 20 parts of crystalline sodium sulfate are added after 10 minutes and a further 20 parts thereof after 20 minutes. At the end of this period there are added to the dyebath 20 parts by volume of an aqueous solution containing in 100 parts by volume 10 parts of sodium-copper pyrophosphate, and the treatment is continued for 30 minutes. The dyebath is then well exhausted. The dyeing is rinsed in the cold, centrifuged and dried. There is obtained an orange-yellow dyeing of good fastness to light and washing.

By using instead of the aforesaid sodium-copper pyrophosphate solution the same quantity of a solution of 4.28 parts of crystalline copper sulfate and 15.4 parts of crystalline tetrasodium pyrophosphate in 90 parts of water, the dyeing process gives a similar result.

A similar result is obtained by using, instead of sodium-copper pyrophosphate, sodium-nickel pyrophosphate or a mixture of solution of equimolecular quantities of nickel sulfate and sodium pyrophosphate.

The dyestuff used in this example can be metallized, instead of with the derivatives of pyrophosphoric acid, with sodium-copper tripolyphosphate, hexasodium-copper tetrapolyphosphate and also with sodium-copper hexametaphosphate, or with mixtures which yield these compounds, of copper sulfate and sodium-tripolyphosphate, sodium tetrapolyphosphate or sodium hexametaphosphate.

Sodium-copper tripolyphosphate is prepared as follows:

36.8 parts of anhydrous sodium tripolyphosphate are dissolved in 200 parts of hot water, and the solution is added to a solution of 25 parts of crystalline copper sulfate ( $\text{CuSO}_4 \cdot 5\text{H}_2\text{O}$ ) in 100 parts of water. There is immediately formed a white precipitate of copper tripolyphosphate, which is filtered off and washed with water.

The copper tripolyphosphate so obtained is introduced into a boiling solution of 36.8 parts anhydrous sodium tripolyphosphate in 200 parts of water, and the mixture is boiled until dissolution is complete. The blue clear solution is evaporated in vacuo, and the easily soluble sodium-copper tripolyphosphate is obtained as a blue powder.

By using, instead of sodium tripolyphosphate an

equimolecular quantity of hexasodium tetrapolyphosphate the corresponding hexasodium-copper polyphosphate is obtained.

Sodium copper hexametaphosphate is prepared as follows:

62 parts of anhydrous sodium hexametaphosphate are dissolved in 300 parts of hot water, and the solution is added to a solution of 25 parts of crystalline copper sulfate ( $\text{CuSO}_4 \cdot 5\text{H}_2\text{O}$ ) in 100 parts of water. The blue clear solution is then evaporated in vacuo, and the easily soluble sodium-copper hexametaphosphate is obtained as a blue powder. Instead of the above mentioned sodium salts of the said phosphoric acid the corresponding potassium can be used.

15 Instead of using the dyestuff of the above formula, the following dyestuffs may be used for dyeing cotton, linen or rayon in the manner described in this example:

|   |  | Dyestuff of the formula                                                              | Tint of dyeing                               |
|---|--|--------------------------------------------------------------------------------------|----------------------------------------------|
| 1 |  |    | {Cu: Blush grey.<br>(Ni: Greenish blue.      |
| 2 |  |    | {Cu: Blue.<br>(Ni: Navy blue.                |
| 3 |  |    | {Cu: Orange.<br>(Ni: Orange.                 |
| 4 |  |   | {Cu: Brown.<br>(Ni: Brown.                   |
| 5 |  |  | {Cu: Bordeaux.<br>(Ni: Bordeaux.             |
| 6 |  |  | {Cu: Blue.<br>(Ni: Blue.                     |
| 7 |  |  | {Cu: Reddish yellow.<br>(Ni: Reddish yellow. |

What we claim is:

1. Process for dyeing cellulosic materials with metallizable direct dyestuffs, which form sparingly soluble metal complexes, by adding an agent yielding metal to a bath containing at least a small quantity of non-metallized dyestuff, which process comprises adding to the dyebath an agent yielding a metal having an atomic number from 28 to 29 and carrying out the metallization in a neutral to alkaline medium in the presence of anions of a polyphosphoric acid and in the absence of amines.

2. Process for dyeing cellulosic materials with metallizable direct dyestuffs, which form sparingly soluble metal complexes, by adding an agent yielding metal to a bath containing at least a small quantity of non-metallized dyestuff, which process comprises adding to the dyebath an agent yielding a metal having an atomic number from 28 to 29 and carrying out the metallization in a neutral to alkaline medium in the presence of anions of a polyphosphoric acid of the formula



in which  $m$  represents a whole number greater than 1 and in the absence of amines.

3. Process for dyeing cellulosic materials with metallizable direct dyestuffs, which form sparingly soluble metal complexes, by adding an agent yielding metal to a bath containing at least a small quantity of non-metallized dyestuff, which process comprises adding to the dyebath an agent yielding a metal having an atomic number from 28 to 29 and carrying out the metallization in a neutral to alkaline medium in the presence of anions of pyrophosphoric acid and in the absence of amines.

4. Process for dyeing cellulosic materials with metallizable direct dyestuffs, which form sparingly soluble metal complexes, by adding an agent yielding metal to a bath containing at least a small quantity of non-

the dyebath an alkali-Me pyrophosphate, Me representing a metal having an atomic number from 28 to 29 and carrying out the metallization in a neutral to alkaline medium and in the absence of amines.

5. Process for dyeing cellulosic materials with metallizable direct dyestuffs, which form sparingly soluble metal complexes, by adding an agent yielding metal to a bath containing at least a small quantity of non-metallized dyestuff, which process comprises adding to the dyebath an agent yielding copper and carrying out the metallization in a neutral to alkaline medium and in the presence of anions of pyrophosphoric acid provided by the addition of an alkali pyrophosphate and in the absence of amines.

10 15. Process for dyeing cellulosic materials with metallizable direct dyestuffs, which form sparingly soluble metal complexes, by adding an agent yielding metal to a bath containing at least a small quantity of non-metallized dyestuff, which process comprises adding to the dyebath an alkali-copper pyrophosphate and carrying out the metallization in a neutral to alkaline medium and in the absence of amines.

15 20. Process for dyeing cellulosic materials with metallizable direct dyestuffs, which form sparingly soluble metal complexes, by adding an agent yielding metal to a bath containing at least a small quantity of non-metallized dyestuff, which process comprises adding to the dyebath an alkali-nickel pyrophosphate and carrying out the metallization in a neutral to alkaline medium and in the absence of amines.

20 25. Process for dyeing cellulosic materials with metallizable direct dyestuffs, which form sparingly soluble metal complexes, by adding an agent yielding metal to a bath containing at least a small quantity of non-metallized dyestuff, which process comprises adding to the dyebath an alkali-copper pyrophosphate and carrying out the metallization in a neutral to alkaline medium and in the absence of amines.

25 30. Process for dyeing cellulosic materials with metallizable direct dyestuffs, which form sparingly soluble metal complexes, by adding an agent yielding metal to a bath containing at least a small quantity of non-metallized dyestuff, which process comprises adding to the dyebath an alkali-nickel pyrophosphate and carrying out the metallization in a neutral to alkaline medium and in the absence of amines.

30 35. Process for dyeing cellulosic materials with metallizable direct dyestuffs, which form sparingly soluble metal complexes, by adding an agent yielding metal to a bath containing at least a small quantity of non-metallized dyestuff, which process comprises adding to the dyebath wherein the dyestuff of the formula



metallized dyestuff, which process comprises adding to the dyebath an agent yielding a metal having an atomic number from 28 to 29 and carrying out the metallization in a neutral to alkaline medium in the presence of anions of hexametaphosphoric acid and in the absence of amines.

5. Process for dyeing cellulosic materials with metallizable direct dyestuffs, which form sparingly soluble metal complexes, by adding an agent yielding metal to a bath containing at least a small quantity of non-metallized dyestuff, which process comprises adding to the dyebath an agent yielding a metal having an atomic number from 28 to 29 and carrying out the metallization

is for the most part fixed on the material to be dyed, sodium-copper hexametaphosphate and carrying out the metallization in a neutral to alkaline medium and in the absence of amines.

50 11. Process for dyeing cellulosic materials with metallizable direct dyestuffs, which form sparingly soluble metal complexes, by adding an agent yielding metal to a bath containing at least a small quantity of non-metallized dyestuff, which process comprises adding cupric sulfate to the dyebath before the material to be dyed is entered, which dyebath contains sodium pyrophosphate and the dissolved dyestuff of the formula



in a neutral to alkaline medium and in the presence of anions of pyrophosphoric acid provided by the addition of an alkali pyrophosphate and in the absence of amines.

6. Process for dyeing cellulosic materials with metallizable direct dyestuffs, which form sparingly soluble metal complexes, by adding an agent yielding metal to a bath containing at least a small quantity of non-metallized dyestuff, which process comprises adding to

70 and carrying out the metallization in a neutral to alkaline medium and in the absence of amines.

12. Process for dyeing cellulosic materials with metallizable direct dyestuffs, which form sparingly soluble metal complexes, by adding an agent yielding metal to a bath containing at least a small quantity of non-metallized dyestuff, which process comprises adding sodium-copper pyrophosphate to the dyebath before the

material to be dyed is entered, which dyebath contains the dissolved dyestuff of the formula



and carrying out the metallization in a neutral to alkaline medium and in the absence of amines.

13. Process for dyeing cellulosic materials with metalizable direct dyestuffs, which form sparingly soluble metal complexes, by adding an agent yielding metal to a bath containing at least a small quantity of non-metallized dyestuff, which process comprises adding sodium-copper pyrophosphate to the dyebath before the

and carrying out the metallization in a neutral to alkaline medium and in the absence of amines.

14. Process for dyeing cellulosic materials with metal-lizable direct dyestuffs, which form sparingly soluble metal complexes, by adding an agent yielding metal to a bath containing at least a small quantity of non-metallized dyestuff, which process comprises adding sodium-nickel pyrophosphate to the dyebath before the material to be dyed is entered, which dyebath contains the dissolved dyestuff of the formula.



material to be dyed is entered, which dyebath contains the dissolved dyestuff of the formula



and carrying out the metallization in a neutral to alkaline medium and in the absence of amines.

**References Cited in the file of this patent**

UNITED STATES PATENTS

- |           |        |               |
|-----------|--------|---------------|
| 2,148,659 | Straub | Feb. 28, 1939 |
| 2,185,905 | Straub | Jan. 2, 1940  |
| 2,243,020 | Straub | May 20, 1941  |

## FOREIGN PATENTS

- 445.466 Great Britain ----- Apr. 14, 1936

#### OTHER REFERENCES

Ind. and Eng. Chem., for November 1951, p. 5A (advertisement).

American Dyestuff Reporter, for January 28, 1935,  
pp. 40 to 47.